

April 15, 1930.

A. C. FISCHER

1,755,108

PREFORMED RAIL FILLER

Filed June 30, 1927



Inventor:  
Albert C. Fischer  
By Ballard Moore attorney

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## PREFORMED RAIL FILLER

Application filed June 30, 1927. Serial No. 202,581.

My invention relates to a preformed rail filler comprising a prepared strip of waterproofing material, preferably bituminous material or other suitable binder shaped to conform to the outline of the rail on one side and suitably faced for contact with the paving on the other side, the strip being adapted to act as insulating, sound-deadening, and expansion material, deadening the sound of the car upon the rail and insulating the track from the adjacent paving material and taking up expansion and contraction between them.

My invention is concerned more with the substance out of which the strips are made rather than to their particular form.

One of the objects of my invention resides in providing a preformed rail filler comprising waterproofing binder and linear fibres which are suitably interlocked or felted together, not only to assist in the insulating and sound deadening characteristics of the strip and providing an efficient flow retarder for the compressible waterproofing binder, such as bituminous material, but also providing an efficient structural reinforcing medium for the rail filler, and in addition considerably to augment the expansibility and compressibility and sound deadening efficiency of the strip.

These and other objects of my invention will be apparent from a perusal of the following specification when taken in connection with the accompanying drawings, wherein,

Figures 1 to 6 inclusive illustrate various designs of strips which may be used singly or collectively in connection with a rail after the manner illustrated and claimed in an application filed January 6, 1926, by H. W. Herbst, Serial No. 79,543.

It is understood that any of the blocks or strips shown in the application aforesaid, or any other type of strip may be availed of, the present invention being concerned with the material of which the rail filler strips are composed.

In this invention I propose to form my rail filler of a mixture of waterproofing material, such as, bituminous material, prefer-

ably blown bituminous material, and interlocking linear fibres of any desired type; they must have length as distinguished from finely divided material which constitutes the cheap filler and flow retarder at present being used. The linear fibres are suitably mixed with the bituminous material when the latter is in the liquid state, in a suitable mixing machine, and then the mixture is extruded, molded, rolled or pressed into suitable form. The linear fibres should not exceed twenty five per cent.

In certain instances I may add earthy or mineral material since it facilitates the extrusion and provides a cheap filler. These earthy materials may include limestone dust, slate particles, infusorial earth, clay and others, and may be used in amounts from ten to twenty per cent.

The interlocking linear fibres which are used in my present invention are of any kind provided they have length as distinguished from sawdust, shredded wood, granular fibrous material and the like, which latter constitute a cheap filler but lack the reinforcing qualities which provide a most valuable component of my rail filler. In addition the linear fibres improve the sound deadening qualities, whereas the finely divided cheap fillers heretofore used detract from the sound deadening qualities of the filler.

The great value of my improved rail filler as differing from types heretofore disclosed, resides in the internal structure of the interlocked fibers, which form an internal mat structure within the rail filler, which adds strength and body and resists flowing of the binder, and in addition is of such a structure that it will stand up as a fibre mat even after the binder has been removed therefrom.

The linear fibres which I use in connection with my invention may be of any desired kind provided they have length so as to permit them to interlock when mixed with the waterproof binder.

In certain instances I propose to use fibres that are cellular in nature. Excelsior fibres are an example of such cellular fibres.

In certain instances also I can prepare my preferred rail filler wherein the linear fibres

are either saturated or not saturated with the binder. This may include a number of variations, for instance, when the fibres themselves are cellular to a certain degree, by mixing them with the bituminous material while in a hot plastic state and limiting the temperature and the period of mixing, the saturation of the cells of the fibres can be avoided so that the fibres retain their inherent and pristine compressibility, whereas by mixing these same fibres at higher temperatures and for longer periods the bituminous binder will thoroughly saturate the fibres.

15 In another sense, I can form the rail filler either saturated or unsaturated with the binder. For instance, I do not use this term "saturated" solely to convey the idea that the fibres of mineral wool or asbestos and the 20 like are saturated. As a matter of fact, it is substantially impossible to saturate mineral wool or asbestos fibres, but when these fibres are felted, the interstices formed by the loosely matted fibres may perhaps be filled so that the 25 filled structure becomes saturated. By simply loosely felting the fibres into a block-like structure, I am able to fill the mass with the waterproofing substance so that a great many of the fibres are separated from each 30 other by a substantial thickness of waterproofing material.

As a modified form, in the event that I desire to produce a very much lighter structure, I use the waterproofing substance in a 35 very much thinner consistency, so that the surplus drains off and thus leaves unfilled interstices between the fibres. This produces a cellular construction.

Should I desire to produce a cellular structure, but with the fibres more closely compacted, I express the surplus saturant and thus leave a cellular structure with the fibres more closely compacted.

I have discovered that mineral wool fibres 45 are cellular, and excelsior and other fibres are also cellular. Consequently I think it best to make some distinction between a structure in which the cells are derived from leaving interstices between the fibres when the 50 same are felted and a structure in which the fibres themselves are cellular. In this connection I call attention to the fact that by using mineral wool, or other fibres which are cellular, I may still produce a cellular structure 55 and at the same time fill the interstices between the fibres in the matted mass. On the other hand, if I do not fill the interstices between the fibres in the matted mass I increase the cells in the structure so that a 60 very highly compressible matted structure is produced. With these conclusions it will be seen that by mixing cellular fibres and a goodly quantity of waterproofing substance, such as asphalt, in the hot plastic state, I 65 produce a more or less solid structure and at

the same time take advantage of the cells in the fibres to develop a more or less high degree of compressibility and expansibility.

On the other hand, by using a very light waterproofing saturant I can increase this compressibility and expansibility by simply matting the fibres together and leaving the interstices to develop the cell structure and also take advantage of the cells in the fibres themselves.

As a modification by using cellular fibres and highly heated bituminous material the latter will saturate the cells of the fibres.

It can readily be understood that the incorporation of the described interlocking linear fibrous material in the waterproofing or bituminous material will insulate any of the granite, concrete or brick paving over the rail, and the fibrous structure will take up the sound and prevent its transmission from the rail to the hard paving substances. Furthermore, the binder, with the aid of the interlocking linear fibres will also provide a suitable expansion joint, due to the compressible qualities not only of the bituminous material but also due to the resiliency of the fibrous material mixed therewith and particularly when the fibrous material is in an unsaturated state as hereinbefore stated.

I claim:

1. A preformed rail filler adapted as an expansion, sound deadening and insulating material, comprising a waterproof binder, linear fibres, and slate particles.

2. A preformed rail filler adapted as an expansion, sound deadening and insulating material, comprising a waterproof binder, linear fibres and earthy material, said fibres being interlaced to reinforce the binder.

3. A preformed rail filler adapted as an expansion, sound deadening and insulating material, comprising bituminous material and interlocked linear fibres not exceeding twenty-five per cent.

4. A preformed rail filler adapted as an expansion, sound deadening and insulating material, comprising bituminous material, interlocked linear fibres, and earthy material in amount from ten to twenty per cent.

5. A preformed rail filler adapted as an expansion, sound deadening and insulating material, comprising a bituminous binder, linear fibres, and slate particles.

6. A preformed rail filler adapted as an expansion joint, sound deadener and insulating material, comprising a bituminous binder, linear fibers and earthy material, said fibres being interlaced to reinforce the bituminous binder.

Signed at Chicago, Illinois, this 16th day 125 of June, 1927.

ALBERT C. FISCHER.

70

75

80

85

90

95

100

105

110

115

120

125

130